

## UNITED STATES PATENT OFFICE

2,267,753

PROCESS OF PREPARING PLATINUM ALLOY  
CATALYSTS FOR GAS REACTION AND THE  
CATALYSTS OBTAINABLE THEREBYKonrad Ruthardt, Hanau, Germany, assignor to  
I. G. Farbenindustrie Aktiengesellschaft, Frank-  
fort-on-the-Main, GermanyNo Drawing. Application January 6, 1939, Serial  
No. 249,590. In Germany December 31, 1936

12 Claims. (Cl. 252—234)

The present invention relates to a process of preparing highly active platinum alloy catalysts and to the catalysts obtainable thereby.

Numerous methods have been suggested for the industrial oxidation of ammonia and for other gas reactions in which pressure, temperature and the arrangement of the apparatus vary. As catalysts there are preferably used platinum metals and alloys of different platinum metals or of platinum metals with other metals suitable for this purpose. The reaction is rapidly started by platinum itself. In the case of other catalysts, for instance alloys of platinum and rhodium, the catalysts begin to work satisfactorily only after several days, as the catalyst is activated by the reaction of the ammonia itself only after a certain time of this reaction, which activation is accompanied by a roughening and sprouting of the surface. Alloys like the known alloys of platinum and ruthenium could hitherto not be used as catalysts in the oxidation of ammonia, for no activation occurs with them while in contact with the ammonia. By many other metals likewise the activation of the alloys is prevented under usual operating conditions.

It is an object of this invention to render useful for catalysts the alloys containing platinum with other metals which under ordinary working conditions and the methods of the activation usual in this case start the reaction (of which the combustion of ammonia is an example) either not at all or insufficiently or only after the elapse of some time.

The pre-treatment of the catalysts in the manner hereinafter described is advisable in the case of all alloys which contain at least 50 per cent of platinum and at least one metal selected from the group comprising ruthenium, osmium, iridium, cobalt, nickel, iron, zirconium, thorium, vanadium, niobium, tantalum, chromium, molybdenum, manganese and rhenium, each metal of the said group being present in a quantity of at least 0.1 per cent. According to the present invention these alloys are recrystallized before they are used as catalysts by heating them to such an extent that the formation of crystals may be detected by means of X-rays. It is necessary that the catalysts be in the worked state in order to obtain the desired recrystallization (see pages 102 through 104 of "The Principles of Physical Metallurgy" by Doan, first edition, 1935).

In case the alloys contain platinum and ruthenium, rhodium may be added as a further constituent. Besides platinum and at least one

of the other metals of the afore-said group tungsten may be present in an amount of 0.1 to 30 per cent, if desired together with rhodium.

After having been recrystallized the alloys of the kind described are distinguished by an especially good catalytic action already at reaction temperatures which are essentially lower than those necessary for catalysts of platinum or of platinum and rhodium without obtaining a worse yield. Moreover, the said alloys have a good mechanical stability especially a good tensile strength, even in the heat. The recrystallized alloys are therefore particularly valuable for gas reactions, for they give higher yields than the alloys hitherto known and the losses in weight of the catalyst are smaller, owing to the low reaction temperatures. The catalysts may not only be used for the oxidation of ammonia but also for the synthesis of ammonia, the preparation of hydrocyanic acid from compounds containing carbon and nitrogen according to Andrusow as well as for hydrogenations and dehydrogenations of hydrocarbons, for the oxidation of alcohols so as to form aldehydes, and for other catalytic reactions.

The alloys mentioned could hitherto not be utilized in the industry on a large scale because they had the drawback of insufficiently causing the reaction to begin. If, however, the alloys are recrystallized, the reaction begins after a relatively short time; this is called: the catalyst "is lighted". The period of time until the reaction of ammonia entirely sets in, when non-recrystallized catalysts of the aforesaid kind are used, is a multiple of the time necessary while using the same catalysts in the recrystallized state. In the case of the combustion of ammonia with the aid of recrystallized catalysts, for instance, the reaction sets in after a short time so that even when the catalyst is exchanged the production is hardly retarded. When the new catalysts are used the yields are very high. Besides, the new catalysts, especially those which besides platinum and ruthenium contain at least one further metal of the aforesaid group, are distinguished by favorable mechanical properties and a high stability. This is surprising, for ternary or quaternary alloys generally are of lower mechanical strength than binary alloys.

The new catalysts are obtained by heating the alloys in question above the recrystallization temperature, for instance in an electric furnace. The recrystallization must be continued until crystals have been distinctly formed.

In the preparation of the catalysts by heating

it is not sufficient that the recrystallization has just set in.

The alloys have generally to be heated for at least one hour at a temperature of at least 900° C. but, according to the kind of the alloy, a longer period and a higher temperature may also be necessary. The progress of the recrystallization may be observed by means of X-rays. The process may be performed in the presence of protective gases such as nitrogen.

It has been found that the said alloys recrystallized in this manner are especially useful as catalysts. This is remarkable because the known facts indicate that the catalytic efficacy would be decreased by too strong a development of the crystals. By this heating and a recrystallization any prevention of catalytic force of the alloys is removed.

For alloys with platinum and very small quantities of rhodium an annealing at 2000° F. (about 1100° C.) and a subsequent treatment with acid has already been suggested. These alloys of platinum and rhodium without any further additions do not necessitate an annealing because the alloys only after a relatively short time are spontaneously activated in contact with the ammonia, to be oxidized whereby their surface is roughening and sprouting. The new alloys according to the present invention, however, which contain other constituents are not or only very slowly roughened at the surface and activated by the action of the gas mixture containing ammonia.

The aforesaid activation of the usual catalysts (so-called "formation") which is occasionally observed at raised temperatures on applying these catalysts for gas reactions cannot be compared with the recrystallization according to this invention. The "formation" which always occurs during the reaction to be influenced by the catalyst is only very slow and generally requires days and weeks; it is combined with a deformation of the catalysts mammillary or clustered structures sprouting from the surface of the contact. The "formation" depends on the chemical process of the gas reaction, perhaps it is even a chemical reaction itself. The recrystallization according to the present invention, however, is a physico-metallurgical process which influences only the structure of the contact and lets the surface substantially unaltered. It may even be said that by the previous recrystallization the "formation" is prevented since no "formation" occurs during the recrystallization and, furthermore, merely relatively low temperatures are applied which are not sufficient for the "formation." By the fact that during the recrystallization and the further use of the surface of the contact, the temperature of use which is relatively lower than that of non-recrystallized contacts, is roughened only to a small extent, the danger of losses in metal caused by the current of hot gases is much smaller than in the case of contacts roughened by the "formation" over which contacts the gases stream at high temperatures.

The advantage of the new contacts, therefore, lies in the fact that the gas reactions are activated in a relatively short time, that a better guarantee is given for the starting of the reaction and that the yield attained is better, even at a relatively low temperature, then in the case of non-recrystallized catalysts. A further advantage is that, owing to the rapid "lightening" of the contacts, the temperature of the metal is rather uniform at all parts so that a deforma-

tion, which in the case of the known contacts was inevitable and caused by the irregular distribution of temperature, may hardly occur.

Without this previous recrystallization the alloys start the reaction either not at all or insufficiently and therefore they could hitherto not be applied. The new alloys have quite another behaviour than the known alloys, for instance of platinum and rhodium, which start gas reactions relatively rapidly already without a thermal pre-treatment. The essential feature of the present invention is therefore: (1) the selection of such alloys as have a particularly good catalytic efficacy which, however, in the non-pretreated state of the catalyst is still latent; (2) the exciting of this efficacy by the recrystallization. The combination of these two features constitutes the new invention. The methods known from the use of platinum-rhodium alloys are not applicable for the new catalysts mentioned above, but this special group of alloys necessitates recrystallization in order to become effective.

The catalysts of the recrystallized alloys herein described are applied in the form of foraminous screens, i. e. in the form of gauze, sieves, spirals, perforated plates and the like. They are likewise advantageously used in combination with other catalysts, for instance with catalysts of noble or non-noble metals or oxides and the like.

The following table shows a number of alloys of the kind described and their efficiency as catalysts, but it is not intended to limit the invention thereto. All the catalysts shown in the table are recrystallized by heating them for one hour to a temperature of 980° C. to 1020° C. in an atmosphere of hydrogen.

The table shows also that in the oxidation of ammonia the catalysts of the invention, i. e. the above-named alloys in the recrystallized state, have the same or a better yield than the catalysts hitherto usual. The recrystallized catalysts, therein, have the further advantage that sufficient yields are already attained at about 650° C. whereas with application of the known catalysts the same high yields are only obtained at a temperature of about 800° C. to 900° C. or more.

Moreover, the table shows that some of the alloys (Nos. 1, 3, 6 and 7) are distinguished by a high stability in the heat at the most various temperatures, even after a continual glowing. The kind of the gaseous atmosphere in which the glowing is performed is not important herein.

| No. | Composition of the alloys      | Yield in the oxidation of ammonia at a reaction temperature of about 650° C. | Remarks                                                                           |                                                           |
|-----|--------------------------------|------------------------------------------------------------------------------|-----------------------------------------------------------------------------------|-----------------------------------------------------------|
|     |                                |                                                                              | Percent                                                                           |                                                           |
| 60  | 1 96% Pt+3% Rh+1% Ru           | 95.6                                                                         | Especially high stability in the heat.                                            |                                                           |
|     | 2 97% Pt+2% Os+1% Ru           | 94.0                                                                         |                                                                                   |                                                           |
|     | 3 95.5% Pt+2% Ru+1.5% Ir+1% Rh | 96.1                                                                         |                                                                                   | Finely crystalline—especially high stability in the heat. |
| 65  | 4 99% Pt+1% Os                 | 95.6                                                                         | Finely crystalline—distinguished by an especially high stability in the heat.     |                                                           |
|     | 5 96.5% Pt+2% Ru+1.5% Ir       | 96.0                                                                         |                                                                                   |                                                           |
|     | 6 97% Pt+2% Ru+1% Os           | 96.4                                                                         |                                                                                   |                                                           |
| 70  | 7 97.5% Pt+2% Ru+0.5% Zr       | 95.9                                                                         | Finely crystalline—distinguished by an especially high stability in the heat. Do. |                                                           |
|     | 8 96.5% Pt+0.5% Ru+3% W        | 92.1                                                                         |                                                                                   |                                                           |

The following examples serve to illustrate that

the catalysts of the new alloys become completely active only when recrystallized:

(1) Mixtures of air and ammonia are caused to react at a relatively low temperature (about 750° C.) and under conditions which procure oxidation of 90.2-90.4 per cent of the ammonia, when platinum is used as a catalyst. When nets of an alloy of platinum and 2 per cent of ruthenium are used which has been recrystallized in an electric furnace by heating for several hours to 1000° C., the yields amount to 94.5 per cent, whereas in the case of non-treated alloys of platinum and ruthenium 80 per cent at best of the ammonia is oxidized. The crystals formed may be detected in the recrystallized alloy of platinum and ruthenium by means of X-rays. The nets made of this recrystallized alloy have been found to be particularly stable.

(2) When using for the reaction described in Example 1 a net of an alloy of platinum, 2 per cent of ruthenium and 1 per cent of rhodium practically no combustion of ammonia could be obtained without a longer activating pre-treatment. With the same net treated at 1000° C. a yield of 96.4 per cent was obtained.

The present application is a continuation-in-part of my application Serial No. 133,821.

I claim:

1. A process of preparing highly active platinum alloy catalysts for gas reactions from worked alloys which are normally practically ineffective as catalysts for said gas reactions, said alloys containing at least 50% of platinum and at least .1% of a metal selected from the group consisting of ruthenium, osmium, iridium, zirconium, thorium, vanadium, niobium, tantalum, chromium, molybdenum, manganese and rhenium which comprises heating said alloys prior to contact with said gases to a temperature of at least about 900° C. but below the melting point of the alloy for a period of at least about one hour, the time being greater the lower the temperature, and vice versa, and the time and temperature being so correlated that recrystallization of the alloys may be detected to a substantial extent by means of X-rays.

2. A process of preparing highly active platinum alloy catalysts for gas reactions from worked alloys which are normally practically ineffective as catalysts for said gas reactions, said alloys containing at least 50% of platinum, at least .1% of ruthenium and at least .1% of a metal selected from the group consisting of rhodium, osmium, iridium, cobalt, nickel, iron, zirconium, thorium, vanadium, niobium, tantalum, chromium, molybdenum, manganese and rhenium, which comprises heating said alloys prior to contact with said gases to a temperature of at least about 900° C. but below the melting point of the alloy for a period of at least about one hour, the time being greater the lower the temperature, and vice versa, and the time and temperature being so correlated that recrystallization of the alloys may be detected to a substantial extent by means of X-rays.

3. A process of preparing highly active platinum alloy catalysts for the reactions from worked alloys which are normally practically ineffective as catalysts for said gas reactions, said alloys containing at least 50% of platinum, .1 to 30% of tungsten and at least .1% of a metal selected from the group consisting of ruthenium, rhodium, osmium, iridium, zirconium, thorium, vanadium, niobium, tantalum, chromium, molybdenum, manganese and rhenium, which com-

prises heating said alloys prior to contact with said gases to a temperature of at least about 900° C. but below the melting point of the alloy for a period of at least about one hour, the time being greater the lower the temperature, and vice versa, and the time and temperature being so correlated that recrystallization of the alloys may be detected to a substantial extent by means of X-rays.

10 4. A process of preparing a catalyst for gas reactions from a worked alloy not normally practically effective as a catalyst for said gas reactions, said alloy consisting of 95.5% of platinum, 2% of ruthenium, 1.5% of iridium and 1% of rhodium, which comprises heating said alloy prior to contact with said gases to a temperature of at least about 900° C. but below the melting point of the alloy for a period of at least about one hour, the time being greater the lower the temperature, and vice versa, and the time and temperature being so correlated that recrystallization of the alloy may be detected to a substantial extent by means of X-rays.

20 5. A process of preparing a catalyst for gas

25 reactions from a worked alloy not normally practically effective as a catalyst for said gas reactions, said alloy consisting of 96.5% of platinum, 2% of ruthenium and 1.5% of iridium, which comprises heating said alloy prior to contact with said gases to a temperature of at least about 900° C. but below the melting point of the alloy for a period of at least about one hour, the time being greater the lower the temperature, and vice versa, and the time and temperature being so correlated that recrystallization of the alloy may be detected to a substantial extent by means of X-rays.

30 6. A process of preparing a catalyst for gas reactions from a worked alloy not normally practically effective as a catalyst for said gas reactions, said alloy consisting of 97% of platinum, 2% of ruthenium and 1% of osmium, which comprises heating said alloy prior to contact with

35 said gases to a temperature of at least about 900° C. but below the melting point of the alloy for a period of at least about one hour, the time being greater the lower the temperature, and vice versa, and the time and temperature being so correlated that recrystallization of the alloy may be detected to a substantial extent by means of X-rays.

40 7. A catalyst for gas reactions containing worked alloys not normally practically effective as catalysts for said reactions, said alloys containing at least 50% of platinum and at least .1% of a metal selected from the group consisting of ruthenium, osmium, iridium, zirconium, thorium, vanadium, niobium, tantalum, chromium, molybdenum, manganese and rhenium, said alloys being recrystallized according to the method of claim 1.

45 8. A catalyst for gas reactions containing worked alloys not normally practically effective as catalysts for said reactions, said alloys containing at least 50% of platinum, at least .1% of ruthenium and at least .1% of a metal selected from the group consisting of rhodium, osmium, iridium, cobalt, nickel, iron, zirconium, thorium, vanadium, niobium, tantalum, chromium, molybdenum, manganese and rhenium, said alloys being recrystallized according to the method of claim 1.

50 9. A catalyst for gas reactions containing worked alloys not normally practically effective as catalysts for said reactions, said alloys con-

taining at least 50% of platinum, .1 to 30% of tungsten and at least .1% of a metal selected from the group consisting of ruthenium, rhodium, osmium, iridium, zirconium, thorium, vanadium, niobium, tantalum, chromium, molybdenum, manganese and rhenium, said alloys being recrystallized according to the method of claim 1.

10. A catalyst for gas reactions in the form of a foraminous screen containing worked alloys not normally practically effective as catalysts for said reactions, said alloys containing at least 50% of platinum and at least .1% of a metal selected from the group consisting of ruthenium, osmium, iridium, zirconium, thorium, vanadium, niobium, tantalum, chromium, molybdenum, manganese and rhenium, said alloys being recrystallized by the method of claim 1.

11. A catalyst for gas reactions in the form of a foraminous screen containing worked alloys not normally practically effective as catalysts for 20

said reactions, said alloys containing at least 50% of platinum, at least .1% of ruthenium and at least .1% of a metal selected from the group consisting of rhodium, osmium, iridium, cobalt, nickel, iron, zirconium, vanadium, niobium, tantalum, chromium, molybdenum, manganese and rhenium, said alloys being recrystallized according to the method of claim 1.

12. A catalyst for gas reactions in the form of a foraminous screen containing worked alloys not normally practically effective as catalysts for said reactions, said alloys containing at least 50% of platinum, .1 to 30% of tungsten and at least .1% of a metal selected from the group consisting of ruthenium, rhodium, osmium, iridium, zirconium, thorium, vanadium, niobium, tantalum, chromium, molybdenum, manganese and rhenium, said alloys being recrystallized according to the method of claim 1.

KONRAD RUTHARDT.